

# United States Patent Office

3,086,903

Patented Apr. 23, 1963

1

3,086,903

LEAD PENCIL AND METHOD OF MANUFACTURE  
Harold Grossman, Upper Montclair, N.J., assignor to  
Hassenfeld Bros., Inc., Central Falls, R.I., a corpora-  
tion of Rhode Island  
No Drawing. Filed Apr. 19, 1960, Ser. No. 23,149  
17 Claims. (Cl. 156—273)

The invention relates to improvements in methods for manufacturing lead pencils, and the resultant article. This application is a continuation-in-part of my pending application Serial No. 719,706, filed March 7, 1958, now abandoned.

Leads for wood-encased pencils comprise an extruded mixture of clay and graphite which is baked or sintered at a high temperature, and then impregnated or coated with a grease, wax, oil, or mixture of two or more of such materials to furnish the desired smooth-writing quality. The greasy surface character of the lead makes it difficult to adhere to the surrounding wood sheath. Nevertheless, firm adherence between the lead and the wood is necessary to prevent breakage at the feathered or sharpened writing end, to prevent movement of the lead within the wood sheath, etc. The grooved wood slats are coated or impregnated to furnish added strength, improved resistance to breakage upon sharpening, but bonding the wood slats to each other has not presented any problem. Bonding the greasy lead to the wood, however, has been the subject of intensive research effort for many years.

To the best of my knowledge, it has been necessary to subject the lead to a preliminary treatment of some kind to condition it for adherence to the wood. Essentially, these preliminary conditioning treatments have involved the modification of the greasy surface in some fashion to render the surface suitable for bonding.

One of the early methods for conditioning the greasy lead to prepare it for adherence to the wood is disclosed by Gonzalez, Patent No. 1,892,508, December 27, 1932, and involves immersion of the leads in sulfuric acid, followed by immersion in a solution of a suitable salt, such as calcium chloride, to precipitate the salt onto the lead. The insoluble precipitate formed on the surface of the lead permits adherence to the wood with the usual water soluble glue.

As disclosed in my Patent 1,958,194, January 1, 1935, the greasy lead is prepared for bonding to the wood by treatment with chromic acid, followed by washing in water and neutralization of traces of the chromic acid.

As disclosed in Chesler 2,116,217, May 3, 1938, the greasy lead is treated with a wetting or penetrating agent, such as a sulfonated oil, to provide a surface which is miscible with the water soluble glue used to adhere the wood slats to each other and to the thus treated lead.

Herstein 2,098,452, November 9, 1935, forms crystals of a detergent salt on the surface of the greasy lead, such crystal structure affording mechanical means for keying the thus treated lead to the wood by a water soluble glue.

The surface of the greasy lead has been variously roughened or pitted to permit mechanical keying to the wood by the glue or adhesive. Such surface roughening has been accomplished by a knurled tool or by sand blasting, as disclosed by Ferst 2,131,657, September 27, 1938; by including a gas liberating agent in the composition comprising the lead writing element, the gas, when liberated, providing a pitted surface, as disclosed by Zuckert 2,190,518; by subjecting the greasy lead to an electric arcing action, as shown by Best 2,229,633, January 28, 1941; and by subjecting the greasy leads to an electrochemical action, as disclosed by McKee 2,228,772, January 14, 1941.

2

More recently, and as disclosed by Grieco 2,515,118, July 11, 1950, an adhesive pattern is printed onto the lead prior to impregnation with the essential greasy substance. The adhesive pattern printed lead is then impregnated with a greasy substance. The resulting discontinuous greasy surface, broken up by the printed adhesive pattern, facilitates bonding such conditioned lead to the wood sheath members and the wood sheath members to each other by the same kind of adhesive used to print the pattern on the leads; for example, a vinyl resin emulsion, or other types of adhesives.

It will be apparent that the prior art necessity to resort to a preliminary conditioning of the lead, whether the lead is treated after it has been grease impregnated, or specially treated, as by the pattern printing, before grease impregnation, constitutes an additional operation or operations, and adds to the cost of manufacturing the product.

Moreover, even with the leads preliminarily treated for the purpose of enabling them to be bonded to the wood, the operation of assembling and adhering the leads within the grooved wood slats has been a bottleneck in the process of manufacture. It has been the practice to apply a water soluble animal glue, or any other suitable adhesive, such as a water emulsion of a synthetic resin to the grooved sides of a pair of slats, lay the leads in the grooves of one of the wet coated slats, place the other wet coated slat thereon to form a so-called block, take a plurality of the blocks, anywhere from 40 to 80, place them under pressure in a large clamp, and then put the clamped blocks in a drying oven for a period of approximately six (6) to eight (8) hours in order to set the wet glue line. The unduly long period of time required to dry and set the adhesive to adhere the elements together is in marked contrast to the prior and subsequent rapid operations of grooving the slats, and cutting the blocks and shaping to form the individual pencils. The inordinate amount of time required to assemble and adhere the leads within the blocks has prevented the realization of a straight-line or continuous method of pencil manufacture.

A primary object of the invention is to provide a method of manufacturing wood-encased lead pencils by adhering the leads directly to the wood sheath members or slats, with the leads in their usual greasy condition, unmodified by a preliminary treatment of any kind, either after or before grease impregnation, thereby providing a novel product wherein the greasy lead is adhesively united directly to the wood sheath without any modification of the lead's greasy surface other than may result from the effect of the adhesive itself, which also unites the wood sheath members.

Another important object of the invention is to provide a continuous, or straight-line method of pencil manufacture in the sense that the time interval required to firmly bond the leads within the block or to the wood slats is accomplished substantially as rapidly as the previous operation of grooving the slats and the subsequent operations of cutting the block into individual pencils and suitably shaping such cut units.

These, and other objects and advantages of the invention, will be apparent from the following detailed description of a preferred embodiment of the invention and several modifications thereof.

In accordance with a preferred form of the invention, a pair of grooved wood slats are coated on their grooved sides with a vinyl resin compound in a suitable vehicle or carrier; that is to say, a water emulsion or a solvent solution of the resin. The resin emulsion or solution is applied by brushing or spraying, and the coatings are applied within the grooves as well as on the intervening flat surfaces. The water or solvent is immediately and rapidly driven

off by applying heat to the coatings to form a thin, substantially dry film of the vinyl resin adhesive on each of the grooved slats. Although any suitable heat source may be used, it is preferred to use infra-red lamps. Depending upon the amount of plasticizer present, the temperatures of the vinyl resin films are approximately 100 to 200° C. The leads are placed in the grooves of one of the slats, and while the adhesive films are still hot from the heat of drying, the other slat is placed thereon and the block is subjected to pressure or clamped. Within a period as short as fifteen (15) seconds, the block may be removed from the clamp, and the leads are firmly adhered to the wood, and, of course, the wood slats are also firmly bonded to each other. And this is accomplished with grease impregnated leads of the usual variety, which are in no way conditioned to change their continuous greasy surface characteristics prior to being placed in the grooves of a slat.

Instead of drying the wet coating on the grooved sides of the wood slats before assembling the wood slats with the leads, the slats, with the coatings thereon still wet, may be assembled with the greasy leads in the mating grooves. The coatings are then dried in the absence of any pressure upon the assembly. The assembly is subjected to dielectric or high frequency heating to cause the vehicle or carrier for the vinyl resin adhesive to be driven off. The assembly having the dry line of adhesive is then subjected to pressure in the presence of heat. Additional heating is unnecessary if pressure is applied to the assembly while the dry vinyl resin adhesive film is still hot from the heat of drying.

The preferred vinyl resin adhesive coating composition is a water emulsion of a plasticized vinyl acetate. From the standpoint of the degree of adhesion between the greasy lead and the wood, coupled with the most rapid method of processing and least expense, I have obtained the best results by using a water emulsion of polyvinyl acetate and a plasticizer known as Hercoflex 900, made by the Hercules Powder Company, which is understood to be a benzoic acid derivative. Examples of benzoic acid derivatives are ethylene glycol dibenzoates, and the polyethylene glycol dibenzoates. The solids content of the emulsion is preferably approximately 50%, with a resin content of 80 to 95%, and a plasticizer content of from 5 to 20% by weight. Other known plasticizers, such as a phthalic acid derivative, a glycol derivative, an abietic acid derivative, or an adipic acid derivative may be used. While a water emulsion of the polyvinyl acetate is preferred, a solvent solution may also be used, suitable solvents being alcohol, a chlorinated hydrocarbon, a fatty acid ester, an aromatic hydrocarbon, or a ketone.

The adhesive coating composition may be in the form of a solvent solution of polyvinyl chloride, or a vinyl chloride acetate copolymer, suitably plasticized.

I am unable to definitely account for the phenomenon which enables the achievement of the unusually high degree of adhesion between the greasy, untreated lead and the wood with the plasticized polyvinyl adhesive, when such adhesive is used in the manner as above described. My experimentation has indicated that when an emulsion or solution of the same vinyl composition is used in the usual manner; that is to say, applying pressure to and drying the assembly or block of greasy leads in the grooved wood slats with the line of adhesive in the usual wet condition, the result is poor or no adhesion, regardless of the amount of pressure, and however long the block is clamped and dried. On the other hand, when the adhesive coating is in substantially dry condition prior to clamping or applying pressure to the block, adhesion takes place, in the presence of heat, despite the greasy surface character of the lead. Then, too, the vinyl compounds apparently are peculiarly constituted to afford a satisfactory bond to greasy lead, when used in the manner described. Experimentation with a variety of other thermoplastic adhesive coatings, even when used in the exact same way as herein-

before described, has resulted in poor adhesion. Besides the excellent adhesion furnished by the plasticized polyvinyl compounds when used in the manner described, such compounds furnish an adhesive line which does not unduly dull the cutters when the blocks are cut into the individual pencil units.

The method as hereinbefore described in detail, produces a wood-encased pencil of top quality from the standpoint of the high measure of adhesion between the 10 greasy lead and the wood and, of course, the wood to wood. The method of manufacture is economically advantageous, because the greasy leads do not require a preliminary or special treatment to condition them for bonding to the wood. Also, the rapidity with which the 15 grooved wood slats and the greasy leads may be satisfactorily adhered eliminates the inordinately long period of time heretofore required to clamp and dry the blocks, thereby permitting a straight-line or continuous method of manufacturing pencils.

20 While the particular method hereinbefore described is preferred, numerous modifications may be made to realize some, if not all, of the many advantages over the prior art. For example, while rapidity of processing is best realized by utilizing the same heat of drying the 25 plasticized polyvinyl coatings to adhere the greasy leads to the wood and the wood slats to each other, I have found that a product of substantially equal quality is obtained by first drying the adhesive coatings on the slats to room temperature, and then activating the dried 30 adhesive coatings by applying heat thereto just prior to forming the block, or by applying heat with the pressure applied to the block. Since in this modified form of the invention, the heat of drying is not used to laminate the elements, the coatings may be initially dried 35 without heat, or by the circulation of air.

While the best results are obtained by applying the plasticized polyvinyl emulsion or solution to both grooved slats, it is within the scope of the invention to apply such adhesive coating to only one of the slats before drying, leading, forming the block and applying pressure thereto in the presence of heat. Also, the greasy leads may be placed in the grooves of one of the slats 40 before applying the plasticized polyvinyl coatings to both slats, drying and assembling. Also, while it is most convenient to apply the vinyl resin as a wet coating, the resin may be applied as a dry powder and fused by heat to form the continuous adhesive film or films on one or both grooved sides of the slats.

45 While the invention has been specifically described in connection with greasy leads of the black element type, it is also within the purview of the invention to use leads of the colored type. Colored leads, which generally comprise a suitable pigment or dye, a wax, and a water soluble gum are also difficult to adhere to wood, because 50 of their waxy or greasy-like surface character. The described procedure satisfactorily adheres colored leads to the wood sheath members, and does not require any preliminary treatment of such leads. In processing colored leads, the plasticizer content is increased so that 55 there are approximately equal parts, by weight, of the vinyl resin and the plasticizer.

The term "greasy lead" as used in the claims is intended to include both the black and colored writing lead elements, which have a continuous greasy or waxy surface character, unmodified by any treatment prior to 60 assembly with the slats to change their usual unbroken greasy or waxy surface character for the purpose of obtaining adhesion.

65 It is believed that the numerous advantages of the invention as hereinbefore described, will be apparent from the foregoing detailed description. While a preferred embodiment of the invention has been described, and several modifications have been indicated, it will be apparent that other changes are contemplated within the 70 75

5

spirit and scope of the invention, as sought to be defined in the following claims.

I claim:

1. A method of making wood-encased lead pencils comprising providing a substantially dry vinyl resin adhesive film within the grooves and upon the adjacent flat areas of a grooved wood slat which is assembled with a second grooved slat and with greasy leads disposed in the mating grooves, and applying pressure to the assembly in the presence of heat to directly adhere the greasy leads to a wood slat and the wood slats to each other.

2. A method of making wood-encased lead pencils comprising applying a wet coating of a vinyl resin within the grooves and upon the adjacent flat areas of each of a pair of grooved wood slats, disposing greasy leads in one of the slats, assembling the other slat therewith, and applying pressure to the assembly in the presence of heat to directly adhere the greasy leads to the wood slats and the wood slats to each other, said coating being dried to provide a substantially dry vinyl resin adhesive prior to the application of pressure.

3. A method of making wood-encased lead pencils as set forth in claim 2, wherein the substantially dry vinyl resin adhesive is deposited from an emulsion of plasticized polyvinyl acetate.

4. A method of making wood-encased lead pencils as set forth in claim 2, wherein the substantially dry vinyl resin adhesive is deposited from an emulsion of polyvinyl acetate plasticized with a benzoic acid derivative in the proportions of approximately 80 to 95 percent of the polyvinyl acetate and 5 to 20 percent of the benzoic acid derivative, by weight.

5. A method of making wood-encased lead pencils comprising providing a substantially dry vinyl resin adhesive film within the grooves and upon the adjacent flat areas of a grooved wood slat, assembling the adhesive film coated slat with a second grooved slat and with greasy leads disposed in the mating grooves, and applying pressure to the assembly in the presence of heat to directly adhere to the greasy leads to a wood slat and the wood slats to each other.

6. A method of making wood-encased lead pencils comprising applying a wet coating of a vinyl resin within the grooves and upon the adjacent flat areas of a grooved wood slat, drying the coating to form a substantially dry vinyl resin adhesive film, assembling the adhesive film coated slat with a second grooved slat and with greasy leads disposed in the mating grooves, and applying pressure to the assembly in the presence of heat to directly adhere the greasy leads to a wood salt and the wood slats to each other.

7. A method of making wood-encased lead pencils comprising applying a wet coating of a vinyl resin within the grooves and upon the adjacent flat areas of each of a pair of grooved wood slats, drying the coatings to form a substantially dry vinyl resin adhesive film on each of the slats, disposing greasy leads in one of the slats, placing the other slat thereon, and applying pressure to the assembly in the presence of heat to directly adhere the greasy leads to the wood slats and the wood slats to each other.

8. A method of making wood-encased lead pencils as set forth in claim 7, wherein the substantially dry vinyl resin adhesive film on each of the slats is deposited from an emulsion of plasticized polyvinyl acetate.

9. A method of making wood-encased lead pencils as set forth in claim 7, wherein the substantially dry vinyl resin adhesive film on each of the slats is deposited from an emulsion of polyvinyl acetate plasticized with a benzoic

acid derivative in the proportions of approximately 80 to 95 percent of the polyvinyl acetate and 5 to 20 percent of the benzoic acid derivative, by weight.

10. A method of making wood-encased lead pencils comprising applying a wet coating of a vinyl resin within the grooves and upon the adjacent flat areas of each of a pair of grooved wood slats, applying heat to the coated slats to form a substantially dry vinyl resin adhesive film on each of the slats and, while the coatings are still hot from the heat of drying, placing the other slat thereon and applying pressure to the assembly to directly adhere the greasy leads to the wood slats and the wood slats to each other.

11. A method of making wood-encased lead pencils as  
15 set forth in claim 10, wherein the dry vinyl resin adhesive  
film on each of the slats is deposited from an emulsion of  
plasticized polyvinyl acetate.

plasticized polyvinyl acetate.

12. A method of making wood-encased lead pencils as set forth in claim 10, wherein the substantially dry vinyl resin adhesive film on each of the slats is deposited from an emulsion of polyvinyl acetate plasticized with a benzoic acid derivative in the proportions of approximately 80 to 95 percent of the polyvinyl acetate and 5 to 20 percent of the benzoic acid derivative, by weight.

25 13. A method of making wood-encased lead pencils comprising applying a wet coating of a vinyl resin within the grooves and upon the adjacent flat areas of a grooved wood slat, assembling the coated slat with a second grooved slat and with greasy leads disposed in the mating 30 grooves, drying the coating in the absence of pressure upon the assembly, and then applying pressure to the assembly in the presence of heat to directly adhere the greasy leads to a wood slat and the wood slats to each other.

Other.

35 14. A method of making wood-encased lead pencils comprising applying a wet coating of a vinyl resin within the grooves and upon the adjacent flat areas of each of a pair of grooved wood slats, disposing greasy leads in one of the slats, assembling the other slat therewith, drying  
40 the coatings in the absence of pressure upon the assembly by high frequency heating, and then applying pressure to the assembly in the presence of heat to directly adhere the greasy leads to the wood slats and the wood slats to each other.

45 15. A method of making wood-encased lead pencils as set forth in claim 14, wherein the dry vinyl resin adhesive film on each of the slats is deposited from an emulsion of plasticized polyvinyl acetate.

16. A method of making wood-encased lead pencils as  
50 set forth in claim 14, wherein the substantially dry vinyl  
resin adhesive film on each of the slats is deposited from  
an emulsion of polyvinyl acetate plasticized with a ben-  
zoic acid derivative in the proportions of approximately  
80 to 95 percent of the polyvinyl acetate and 5 to 20 per-  
55 cent of the benzoic acid derivative, by weight.

17. A method of making wood-encased lead pencils as set forth in claim 14, wherein pressure is applied to the assembly while the dried coatings are still hot from the heat of drying.

**References Cited in the file of this patent**

UNITED STATES PATENTS

2,515,118 Grieco ----- July 11, 1950

#### OTHER REFERENCES

Text on Adhesives: "The Technology of Adhesives," by Del Monte, Reinhold Publishing Co., 330 W. 42nd St., New York 18, N.Y. (Copy in Division 60.)